

## 1

3,145,202

**GELATION INHIBITORS FOR SILICONE OILS**  
 Robert M. Silverstein, Menlo Park, and Frank R. Mayo,  
 Atherton, Calif., assignors to the United States of  
 America as represented by the Secretary of the Air  
 Force

No Drawing. Filed Feb. 13, 1961, Ser. No. 89,081  
 1 Claim. (Cl. 252—49.6)

This invention relates to silicone oils and more particularly to antioxidant additives for use therewith.

In general, lubricant materials employed heretofore were based on petroleum hydrocarbons. However, such materials suffer inherent defects with respect to flammability, ease of oxidation, instability at elevated temperatures, lack of lubricity at low temperatures, and concurrent viscosity changes with temperature changes. The use of silicone oils is also well known and to some extent such oils exhibit characteristics which tend to eliminate the problems encountered with the use of petroleum lubricants. The silicone oils, briefly, are derivatives of various polymeric organosiloxanes such as the alkyl silicones, the aryl-alkyl silicones, and the alkyl silicone halides. These oils are characterized by flat viscosity temperature curves and possess oxidative stability up to approximately 200° C. However, the silicone oils oxidize readily at temperatures in excess of 200° C., becoming gel-like and finally carbonizing to form a hard grit-like material completely unsuitable for lubricating purposes. The recent advent of high speed engines, aircraft and other propulsion devices has created a problem of considerable importance with respect to the lubrication of such devices, especially at the elevated temperatures produced during their operation. The various antioxidant additives relied upon in the past to abrogate the inherent defects of both petroleum oils and the silicone oils have proven to be ineffective at these elevated temperatures. Ineffectiveness of the silicone oils at elevated temperatures is due in most part to the fact that the efficacy of presently used additives declines rapidly at higher temperatures resulting in gelation of the oil.

In accordance with this invention it has been found that the aforementioned ineffectiveness of silicone oils when employed at elevated temperatures can be alleviated to a great extent by employing certain aromatic condensed ring compounds as antioxidant additives.

Therefore, it is the primary object of this invention to provide an improved silicone lubricant.

It is a further object of this invention to provide an improved silicone lubricant which is especially suitable for use at elevated temperatures in excess of 200° C.

## 2

Still another object of this invention is to provide an improved silicone lubricant which exhibits a high resistance to oxidation, especially at elevated temperatures.

Still a further object of this invention is to provide an improved silicone lubricant which exhibits little or no viscosity change with each change of temperature.

Still another object of this invention is to provide antioxidant additives which are particularly suitable for use with silicone oils.

10 The above and still further objects and advantages of this invention will become readily apparent upon examination of the following detailed disclosure of specific embodiments thereof.

15 In a more specific aspect, it has been found that the foregoing objects can be accomplished by the addition of minor amounts of aromatic condensed ring compounds to silicone oils. As a class, those condensed ring compounds having at least three angularly or linearly fused rings have been found to be effective in preventing oxidative degradation of silicone oils at temperatures in excess of 200° C. These additives are sufficiently soluble in silicone fluids at both high and low temperatures to a degree that makes them especially suitable as lubricants at the wide temperature ranges encountered during the 20 operation of high speed aircraft. The condensed aromatic ring compounds of this invention are effective in achieving the desired temperature stability necessary to insure the operational efficiency of the silicone oils.

25 The specific additives which have been found to be effective in retarding the gelation or oxidative degradation of silicone oils are disclosed in Table II. These additives were tested, as to their effectiveness in retarding oxidative degradation or gelation of silicone fluids, at 518° F. with dry air at 550° F. with a gaseous mixture of 5 percent O<sub>2</sub> and 95 percent N<sub>2</sub>. These additives were also tested in a similar manner with silane fluid lubricants, naphthenic mineral oils, pentaerythritol tetracaproate fluid lubricants, and paraffinic mineral oils, but were found to be ineffective in retarding oxidation. In 30 order to determine the effectiveness of the antioxidant additives of this invention, air or a gaseous mixture of 95 percent nitrogen and 5 percent oxygen was bubbled through the additive-containing lubricating fluid which in turn was heated to an elevated temperature. Several 35 metal washers were immersed in the fluid in which the antioxidant additive was dissolved. The tabulation set forth in Table I presents the fluids employed and the temperature, duration of test, type of gas, and combination 40 of metal washers for each fluid tested.

Table I  
 TEST CONDITIONS FOR FLUIDS

| Fluid                                     | Temper-<br>ture (° F.) | Time<br>(hr.) | Gas                                    | Washers                                       |
|-------------------------------------------|------------------------|---------------|----------------------------------------|-----------------------------------------------|
| G. E. Versilube, F-50 silicone            | 1 500                  | 48            | Air                                    | Copper, silver, aluminum, steel, titanium.    |
|                                           | 550                    | 48            | 95% N <sub>2</sub> , 5% O <sub>2</sub> | Copper, aluminum, steel, titanium, stainless. |
| Silane, MLO 57-628 <sup>2</sup>           | 500                    | 48            | Air                                    | Copper, silver, aluminum, steel, titanium.    |
|                                           | 550                    | 24            |                                        | Copper, aluminum, steel, titanium.            |
| Paraffinic mineral oil, MLO 57-573        | 500                    | 48            | Air                                    | Copper, silver, aluminum, steel, titanium.    |
|                                           | 550                    | 24            |                                        | Copper, silver, aluminum, steel, titanium.    |
| Naphthenic mineral oil, MLO 57-573        | 550                    | 48            | 95% N <sub>2</sub> , 5% O <sub>2</sub> | Copper, aluminum, steel, titanium, stainless. |
|                                           | 24                     |               |                                        | Copper, aluminum, steel, titanium.            |
| Pentaerythritol tetracaproate, MLO 57-426 | 500                    | 18            |                                        | Copper, silver, aluminum, steel, titanium.    |
|                                           | 500                    | 48            | Air                                    | Copper, silver, aluminum, steel, titanium.    |

<sup>1</sup> Actual temperature was 518° F.

<sup>2</sup> Silane fluid MLO 57-461 was so severely degraded at 500° F. with dry air that testing was discontinued.

Another object of this invention is to provide an improved silicone lubricant which exhibits stability at elevated temperatures.

Table II sets forth the antioxidant additive compounds contemplated by this invention together with test results indicating their overall effectiveness.

Table II

AVERAGE PERCENT VISCOSITY INCREASE AT 100° F. (NUMBER OF RUNS AND APPEARANCE)

| Additive                                  | Additive concentration is highest concentration at which it was soluble at -65° F. |                        |                               | Additive concentration 0.2%  |                               |
|-------------------------------------------|------------------------------------------------------------------------------------|------------------------|-------------------------------|------------------------------|-------------------------------|
|                                           | 518° F.                                                                            | Additive concentration | 550° F.                       | 518° F.                      | 550° F.                       |
| I. 1,2-benzanthracene                     | 22 (2, clear, yellow).                                                             | 0.2                    | 115 (2, dark brown).          | 20 (4, clear, yellow).       | 115 (2, opaque, dark brown).  |
| II. Pyrene                                | 34 (2, clear, dark yellow).                                                        | 0.1                    | 427 (2, dark brown).          | 44 (2, clear, yellow).       | 113 (2, opaque, dark brown).  |
| III. Acenaphthene                         | 41 (2, opaque, brown).                                                             | 1.0                    | 98 (2, opaque, dark brown).   | 105 (2, clear, light brown). | Very viscous (1, dark brown). |
| IV. Phenanthrene                          | 58 (2, clear, yellow).                                                             | 1.0                    | Gel (2, dark brown).          | 68 (3, clear, yellow).       | Gel (1, dark brown).          |
| V. Fluoranthene                           | 97 (2, clear, yellow).                                                             | 0.5                    | Very viscous (2, dark brown). | 85 (5, clear, yellow).       | Gel (2, dark brown).          |
| VI. 2,5-diphenyloxazole                   | Gel (2, brown).                                                                    | 0.5                    | Gel (2, dark brown).          | 51 (4, clear, yellow).       | Gel (1, dark brown).          |
| VII. 1,1'-binaphthyl                      | 56 (1, clear, yellow).                                                             | 0.2                    | Gel (1, dark brown).          | 86 (3, clear, yellow).       | Do.                           |
| VIII. Benzo(a)pyrene <sup>1</sup>         | 18 (2, clear, dark brown).                                                         | 0.2                    | 39 (2, dark brown).           | 16 (3, clear, yellow).       | 38 (2, opaque, dark brown).   |
| XI. Dibenz(a,h)anthracene <sup>1</sup>    |                                                                                    | <0.01                  |                               | 12 (3, clear, light brown).  | 123 (2, opaque, dark brown).  |
| X. Dinaphthylbenzene                      |                                                                                    | <0.01                  |                               | 14 (4, opaque, brown).       | Gel (2, dark brown).          |
| XI. Perylene                              |                                                                                    | <0.01                  |                               | 19 (3, clear, brown).        | 113 (2, opaque, dark brown).  |
| XII. Chrysene                             | 103 (2, clear, yellow).                                                            | 0.03                   | Gel (2, dark brown).          | 68 (2, clear, yellow).       | Gel (1, dark brown).          |
| XIII. Decacylene                          |                                                                                    | <0.01                  |                               | 60 (4, opaque, brown).       | L500 (2, opaque, dark brown). |
| XIV. 4,4'-bis(dimethylamino)-benzophenone | Gel (1, yellow).                                                                   | 0.05                   | Gel (2, dark brown).          | 120 (4, clear yellow).       | Gel (1, dark brown).          |
| XV. Indanthrene Navy Blue BRA Powder      |                                                                                    | <0.01                  |                               | 80 (2, clear, violet).       | Gel (1, violet).              |
| XVI. N-phenylferrocenecarboxamide         |                                                                                    | <0.01                  |                               | 47 (3, opaque, brown).       | Gel (1, black).               |
| XVII. 1,3,5-triphenylbenzene              |                                                                                    | <0.01                  |                               | 720 (2, clear, yellow).      |                               |
| XVIII. 1,12-benzoperylene                 |                                                                                    | <0.01                  |                               | 30 (2, opaque, brown).       |                               |

<sup>1</sup> Potent carcinogen in mice. Due caution in handling should be observed.

As is evident from Table II, the principal criterion for effectiveness was reduction of the viscosity increase in comparison with the fluid containing no additive. Kinematic viscosities were determined at 100° F. and 210° F. Other effects measured were net weight change of fluid, acid number, petroleum ether insolubles, and weight change in metal washers. Oxygen consumption was also determined as well as various oxidative degradation products. The particular silicone fluid used in evaluating the effectiveness of the various antioxidant additives of this invention was General Electric F-50 silicone fluid. This fluid is a dimethylsilicone polymer in which one out of 55 methyl groups were replaced by a 2,3,5,6-tetrachlorophenyl group. End-groups on the silicone polymer chains are trimethylsiloxy groups. The average molecular weight is 3000, corresponding to an average chain length of about 40 units. The F-50 silicone fluid has a fairly low oxygen tolerance at elevated temperatures. When dry air is bubbled through 20 ml. of the unprotected fluid at one liter per hour at 518° F., it gels in an average time of 10.4 hours. The presence or absence of washers had no discernible effect on gel time. At 550° F. with a mixture of 5 percent oxygen and 95 percent nitrogen gel time with washers was 27.8 hours and without washers 23.0 hours. The antioxidant additives were employed at a concentration of 0.2 percent at 518° F. with dry air for 48 hours. At the end of the 48 hour period the unprotected fluid was gelled. A number of the additives contemplated by this invention were able to prevent gelation for this period. At 550° F. with a mixture of 5 percent oxygen and 95 percent nitrogen the unprotected silicone fluids were gelled at the end of the 48 hour period and the gel was discolored and yellow in appearance. The additives of this invention were still effective at 550° F. though less so than at 518° F. in spite of the fact that gel time of the untreated fluid was longer at the higher temperature.

The criteria used to establish additive preference were effectiveness in retarding viscosity increase, low tempera-

ture solubility, appearance of fluid such as darkening or sludging, and toxicity considerations. Gross weight change, acid number, and washer changes did not appear to afford a consistent criteria. None of the effective antioxidants of this invention caused unduly high acid numbers nor did they cause excessive attack on the washers. Effectiveness in retarding viscosity increase was, as stated heretofore, evaluated by kinematic viscosities at 100° F. and 210° F.

Low temperature solubility was determined as follows: The additives were agitated in the fluid at 302° F. with a stream of nitrogen for two hours. The solution was held at room temperature for three days, then at minus 65° F. for three days, and again at room temperature for three days. The additives were then evaluated as antioxidants at the highest concentration at which they were soluble at minus 65° F.

The toxicity factor of some concern was carcinogenic activity. Several of the additives which are effective as antioxidants in silicone fluids exhibit carcinogenic activity, at least in mice, and due care should be exercised in handling such materials.

On the basis of the criteria mentioned above, the additive of choice for silicone fluids is 1,2-benzanthracene. Pyrene is ranked second and acenaphthene third. Fluoranthene, phenanthrene and 2,5-diphenyloxazole are alternate candidates for fourth rank. Acenaphthene was especially effective at 550° F. at a 1.0 percent concentration. The information by which additive preference was determined is summarized in Table II, which in turn is a summation of material taken from Tables III through VI.

For each of the effective compounds Table II sets forth the average percentage viscosity increase at 100° F., the number of runs on which the average was based and the appearance of the fluid after the test. These data are given at two concentration levels. The highest concentration at which the additive was soluble at minus 65° F. and the routine testing level of 0.2 percent. In addition, tests were run at 518° F. with dry air and at 550° F.

with a gaseous mixture of 5 percent oxygen and 95 percent nitrogen. Solubility tests are presented in Table III. The evaluation of the antioxidants in F-50 silicone fluid at their minus 65° F. solubility level is shown at

518° F. in Table IV, and at 550° F. in Table V. Tests results for additive concentration at the 0.2 percent level for 48 hours are shown in Table VI at 518° F., and in Table VII at 550° F.

Table III

SOLUBILITY<sup>1</sup> OF EFFECTIVE COMPOUNDS IN F-50 SILICONE

| Additive                                     | 1.00%          | 0.50% | 0.20% | 0.10% | 0.05% | 0.03% | 0.01% |
|----------------------------------------------|----------------|-------|-------|-------|-------|-------|-------|
| 1,1'-binaphthyl (A):                         |                |       |       |       |       |       |       |
| 2 hours at 150° C. (302° F.)                 | S <sup>3</sup> | S     | S     | S     |       |       |       |
| 3 days at room temp                          | I <sup>3</sup> | I     | S     | S     |       |       |       |
| 3 days at -65° F.                            | I              | I     | S     | S     |       |       |       |
| 3 days at room temp                          | I              | I     | S     | S     |       |       |       |
| Decacyclene (A):                             |                |       |       |       |       |       |       |
| 2 hours at 150° C. (302° F.)                 | I              |       |       |       |       |       | I     |
| 3 days at room temp                          | I              |       |       |       |       |       | I     |
| 3 days at -65° F.                            | I              |       |       |       |       |       | I     |
| 3 days at room temp                          | I              |       |       |       |       |       | I     |
| 1,2-benxanthracene (A):                      |                |       |       |       |       |       |       |
| 2 hours at 150° C. (302° F.)                 | S              | S     | S     |       |       |       |       |
| 3 days at room temp                          | I              | SS    | SS    |       |       |       |       |
| 3 days at -65° F.                            | I              | SS    | SS    |       |       |       |       |
| 3 days at room temp                          | I              | SS    | SS    |       |       |       |       |
| Dinaphthylmethiophene (A):                   |                |       |       |       |       |       |       |
| 2 hours at 150° C. (302° F.)                 | I              |       |       |       |       |       | I     |
| 3 days at room temp                          | I              |       |       |       |       |       | I     |
| 3 days at -65° F.                            | I              |       |       |       |       |       | I     |
| 3 days at room temp                          | I              |       |       |       |       |       | I     |
| 4,4'-bis(dimethylamino) benzophenone (EK):   |                |       |       |       |       |       |       |
| 2 hours at 150° C. (302° F.)                 | I              | S     | S     |       |       |       |       |
| 3 days at room temp                          | I              | I     | SS    |       |       |       |       |
| 3 days at -65° F.                            | I              | I     | SS    |       |       |       |       |
| 3 days at room temp                          | I              | I     | S     |       |       |       |       |
| Chrysene (EK):                               |                |       |       |       |       |       |       |
| 2 hours at 150° C. (302° F.)                 | I              |       |       |       |       |       |       |
| 3 days at room temp                          | I              |       |       |       |       |       |       |
| 3 days at -65° F.                            | I              |       |       |       |       |       |       |
| 3 days at room temp                          | I              |       |       |       |       |       |       |
| N,N'-di-2-naphthyl-p-phenylene-diamine (EK): |                |       |       |       |       |       |       |
| 2 hours at 150° C. (302° F.)                 | I              |       |       |       |       |       | I     |
| 3 days at room temp                          | I              |       |       |       |       |       | I     |
| 3 days at -65° F.                            | I              |       |       |       |       |       | I     |
| 3 days at room temp                          | I              |       |       |       |       |       | I     |
| Indanthrene Navy Blue BRA powder (GD):       |                |       |       |       |       |       |       |
| 2 hours at 150° C. (302° F.)                 | I              |       |       |       |       |       | I     |
| 3 days at room temp                          | I              |       |       |       |       |       | I     |
| 3 days at -65° F.                            | I              |       |       |       |       |       | I     |
| 3 days at room temp                          | I              |       |       |       |       |       | I     |
| 2,5-diphenyloxazole (EK):                    |                |       |       |       |       |       |       |
| 2 hours at 150° C. (302° F.)                 | S              | S     | SS    | S     |       |       |       |
| 3 days at room temp                          | I              | SS    | SS    | SS    |       |       |       |
| 3 days at -65° F.                            | I              | SS    | SS    | SS    |       |       |       |
| 3 days at room temp                          | I              | SS    | SS    | SS    |       |       |       |
| Fluoranthene (RTCC):                         |                |       |       |       |       |       |       |
| 2 hours at 150° C. (302° F.)                 | S              | S     | SS    | SS    |       |       |       |
| 3 days at room temp                          | I              | SS    | SS    | SS    |       |       |       |
| 3 days at -65° F.                            | I              | SS    | SS    | SS    |       |       |       |
| 3 days at room temp                          | I              | SS    | SS    | SS    |       |       |       |
| Perylene (A):                                |                |       |       |       |       |       |       |
| 2 hours at 150° C. (302° F.)                 |                |       | I     | I     |       |       | I     |
| 3 days at room temp                          |                |       | I     | I     |       |       | I     |
| 3 days at -65° F.                            |                |       | I     | I     |       |       | I     |
| 3 days at room temp                          |                |       | I     | I     |       |       | I     |
| Benzo(a)pyrene (EK):                         |                |       |       |       |       |       |       |
| 2 hours at 150° C. (302° F.)                 | S              | S     | SS    | SS    |       |       |       |
| 3 days at room temp                          | I              | I     | SS    | SS    |       |       |       |
| 3 days at -65° F.                            | I              | I     | SS    | SS    |       |       |       |
| 3 days at room temp                          | I              | I     | SS    | SS    |       |       |       |
| Dibenz(a,h)anthracene (EK):                  |                |       |       |       |       |       |       |
| 2 hours at 150° C. (302° F.)                 |                |       | I     | I     |       |       | I     |
| 3 days at room temp                          |                |       | I     | I     |       |       | I     |
| 3 days at -65° F.                            |                |       | I     | I     |       |       | I     |
| 3 days at room temp                          |                |       | I     | I     |       |       | I     |
| Pyrene (CCC):                                |                |       |       |       |       |       |       |
| 2 hours at 150° C. (302° F.)                 | S              | S     | SS    | S     |       |       |       |
| 3 days at room temp                          | I              | I     | SS    | S     |       |       |       |
| 3 days at -65° F.                            | I              | I     | SS    | S     |       |       |       |
| 3 days at room temp                          | I              | I     | SS    | S     |       |       |       |
| Phenanthrene (CCCC):                         |                |       |       |       |       |       |       |
| 2 hours at 150° C. (302° F.)                 | S              |       | S     |       |       |       |       |
| 3 days at room temp                          | S              |       | SS    |       |       |       |       |
| 3 days at -65° F.                            | S              |       | SS    |       |       |       |       |
| 3 days at room temp                          | S              |       | SS    |       |       |       |       |
| Acenaphthene (EK):                           |                |       |       |       |       |       |       |
| 2 hours at 150° C. (302° F.)                 | S              |       | SS    |       |       |       |       |
| 3 days at room temp                          | S              |       | SS    |       |       |       |       |
| 3 days at -65° F.                            | S              |       | SS    |       |       |       |       |
| 3 days at room temp                          | S              |       | SS    |       |       |       |       |
| N-phenylferrocene carboxamide (WADC):        |                |       |       |       |       |       |       |
| 2 hours at 150° C. (302° F.)                 | I              |       |       |       |       |       | I     |
| 3 days at room temp                          | I              |       |       |       |       |       | I     |
| 3 days at -65° F.                            | I              |       |       |       |       |       | I     |
| 3 days at room temp                          | I              |       |       |       |       |       | I     |
| 1,3,5-triphenylbenzene (A):                  |                |       |       |       |       |       |       |
| 2 hours at 150° C. (302° F.)                 |                |       |       |       |       |       | I     |
| 3 days at room temp                          |                |       |       |       |       |       | I     |
| 1,12-benzoperylene (A):                      |                |       |       |       |       |       |       |
| 2 hours at 150° C. (302° F.)                 |                |       |       |       |       |       | I     |
| 3 days at room temp                          |                |       |       |       |       |       | I     |

<sup>1</sup> The additives were agitated in F-50 silicone fluid at 150° C. (302° F.) with a stream of nitrogen for two hours; the solution was held at room temperature for three days, then at -65° F. for three days, and again at room temperature for three days.

<sup>2</sup> A=Aldrich Chemical Co.; EK=Eastman Kodak; GD=General Dyestuff Co.; RTCC=Reilly Tar and Chemical Corporation; CCC=Carbide and Carbon Chemicals Co.; WADC=Wright Air Development Center.

<sup>3</sup> S=soluble. I=insoluble.

Table IV

THE MOST EFFECTIVE COMPOUNDS AT THE HIGHEST CONCENTRATION AT WHICH THEY WERE SOLUBLE AT -65° F.  
IN F-50 SILICONE AT 518° F., 1 LITER DRY AIR/HOUR FOR 48 HOURS

| Additive                                               | Concen-<br>tration,<br>percent | Note-<br>book<br>page | Fluid<br>wt.<br>change<br>(g.) | Viscosity <sup>1</sup> |                                             |                      |                                             | Acid <sup>2</sup><br>No. | Appearance of<br>fluid after test | Change in metals (mg./cm. <sup>2</sup> ) |       |       |                         |       |       |
|--------------------------------------------------------|--------------------------------|-----------------------|--------------------------------|------------------------|---------------------------------------------|----------------------|---------------------------------------------|--------------------------|-----------------------------------|------------------------------------------|-------|-------|-------------------------|-------|-------|
|                                                        |                                |                       |                                | Cs. at<br>100°<br>F.   | Percent<br>visc.<br>change<br>at 100°<br>F. | Cs. at<br>210°<br>F. | Percent<br>visc.<br>change<br>at 210°<br>F. |                          |                                   | Al                                       | Cu    | Steel | Stain-<br>less<br>steel | Ti    | Ag    |
| Phenanthrene<br>(CCC) <sup>3</sup>                     | 1.00                           | 3814-33               | -0.5                           | 90                     | 50                                          | 36                   | 80                                          | 2.1                      | Clear, yellow                     | +0.16                                    | +0.28 | +0.14 | +0.02                   | +0.08 | ----- |
|                                                        | 1.00                           | 3893-4                | -0.5                           | 107                    | 66                                          | 35                   | 75                                          | 1.6                      | do                                | +0.16                                    | +0.14 | +0.08 | +0.02                   | ----- | ----- |
| Acenaphthene (EK)                                      | 1.00                           | 3814-34               | -0.2                           | 81                     | 35                                          | 27                   | 35                                          | 1.8                      | Opaque,<br>brown.                 | +0.08                                    | +0.04 | +0.10 | +0.06                   | +0.02 | ----- |
| 4,4'-bis (di-methyl-<br>amino) benzopheno-<br>ne (EK). | 0.05                           | 3893-5                | -0.4                           | 89                     | 46                                          | 29                   | 45                                          | 2.0                      | Yellow gel                        | +0.04                                    | +0.20 | -0.02 | 0.00                    | +0.10 | ----- |
| Chrysene (EK)                                          | 0.03                           | 3814-36               | -0.8                           | 121                    | 101                                         | 38                   | 90                                          | 1.7                      | Clear, yellow                     | +0.06                                    | 0.00  | +0.04 | -0.16                   | +0.08 | ----- |
| Fluoranthene<br>(RTCC).                                | 0.50                           | 3814-37               | -0.3                           | 123                    | 105                                         | 48                   | 140                                         | 1.8                      | Dark yellow                       | +0.16                                    | +0.12 | +0.12 | +0.04                   | +0.08 | ----- |
|                                                        | 0.50                           | 3893-6                | -0.3                           | 125                    | 69                                          | 29                   | 45                                          | 1.9                      | Clear, dark<br>yellow.            | +0.08                                    | -0.30 | +0.06 | -----                   | +0.04 | +0.24 |
| 2,5-diphenyloxazole<br>(EK).                           | 0.50                           | 3814-38               | -0.4                           | -----                  | -----                                       | -----                | -----                                       | -----                    | Dark brown<br>gel.                | -----                                    | ----- | ----- | -----                   | ----- | ----- |
|                                                        | 0.50                           | 3893-2                | -0.4                           | -----                  | -----                                       | -----                | -----                                       | 1.0                      | Brown gel.                        | -----                                    | ----- | ----- | -----                   | ----- | ----- |
|                                                        | 0.35                           | 3893-9                | -0.3                           | 113                    | 83                                          | 37                   | 85                                          | -----                    | Clear, dark<br>yellow.            | -0.02                                    | -0.32 | +0.02 | 0.00                    | +0.16 | ----- |
| Do                                                     | 0.35                           | 3893-10               | -0.3                           | 487                    | 711                                         | 177                  | 785                                         | 0.9                      | do                                | -0.02                                    | -0.24 | +0.08 | -0.02                   | +0.30 | ----- |
|                                                        | 0.20                           | 3893-11               | -0.1                           | 97                     | 64                                          | 28                   | 40                                          | 1.4                      | Clear, yellow                     | -----                                    | ----- | ----- | -----                   | ----- | ----- |
|                                                        | 0.20                           | 3893-11               | -0.3                           | 119                    | 98                                          | 33                   | 65                                          | 1.2                      | do                                | -----                                    | ----- | ----- | -----                   | ----- | ----- |
|                                                        | 0.10                           | 3814-4                | -0.5                           | 73                     | 21                                          | 28                   | 40                                          | 1.6                      | Clear, light<br>brown.            | +0.06                                    | 0.00  | +0.08 | +0.08                   | +0.06 | ----- |
| Pyrene (CCC)                                           | 0.10                           | 3893-7                | -0.4                           | 88                     | 46                                          | 29                   | 45                                          | 1.9                      | Clear, dark<br>yellow.            | -0.4                                     | -0.10 | +0.16 | -----                   | +0.02 | +0.24 |
| 1,1'-binaphthyl (A)                                    | 0.20                           | 3893-8                | -0.6                           | 94                     | 56                                          | 30                   | 50                                          | 1.9                      | Clear, yellow                     | -----                                    | ----- | ----- | -----                   | ----- | ----- |
| 1,2-benzanthracene<br>(A).                             | 0.20                           | 3814-42               | 0.0                            | 70                     | 16                                          | 23                   | 15                                          | 2.0                      | do                                | -----                                    | ----- | ----- | -----                   | ----- | ----- |
|                                                        | 0.20                           | 3893-8                | -0.4                           | 77                     | 28                                          | 25                   | 25                                          | 2.3                      | do                                | -----                                    | ----- | ----- | -----                   | ----- | ----- |
| Benzo(a)pyrene<br>(EK).                                | 0.20                           | 3814-43               | -0.3                           | 69                     | 15                                          | 24                   | 20                                          | 2.2                      | Clear, dark<br>brown.             | -----                                    | ----- | ----- | -----                   | ----- | ----- |
|                                                        | 0.20                           | 3893-8                | -0.1                           | 72                     | 20                                          | 24                   | 20                                          | 2.1                      | do                                | -----                                    | ----- | ----- | -----                   | ----- | ----- |

<sup>1</sup> Viscosity of F-50 silicone fluid before test was 60 cs. at 100° F. and 20 cs. at 210° F.

<sup>2</sup> Acid number was determined by the procedure given in Scott, Standard Methods of Chemical Analysis, vol. II, page 1844, 5th Ed., 1939, D. Van Nostrand Co., Inc., N.Y.

<sup>3</sup> CCC=Carbide and Carbon Chemicals Co.; EK=Eastman Kodak; RTCC=Reilly Tar and Chemical Corporation; A=Aldrich Chemical Co.

<sup>4</sup> Lower concentrations tested to check observed deleterious effect at higher concentration.

Table V

THE MOST EFFECTIVE COMPOUNDS AT THE HIGHEST CONCENTRATION AT WHICH THEY WERE SOLUBLE AT (-65° F.)  
IN F-50 SILICONE AT 550° F., 1 LITER DRY 5% O<sub>2</sub>-95% N<sub>2</sub>/HOUR FOR 48 HOURS

| Additive                                             | Concen-<br>tration<br>(per-<br>cent) | Note-<br>book<br>page | Fluid<br>wt.<br>change<br>(g.) | Viscosity <sup>1</sup> |                                             |                   |                                             | Acid <sup>2</sup><br>No. | Appearance of<br>fluid after test | Change in metals (mg./cm. <sup>2</sup> ) |       |       |                         |       |       |
|------------------------------------------------------|--------------------------------------|-----------------------|--------------------------------|------------------------|---------------------------------------------|-------------------|---------------------------------------------|--------------------------|-----------------------------------|------------------------------------------|-------|-------|-------------------------|-------|-------|
|                                                      |                                      |                       |                                | Cs. at<br>100° F.      | Percent<br>visc.<br>change<br>at 100°<br>F. | Cs. at<br>210° F. | Percent<br>visc.<br>change<br>at 210°<br>F. |                          |                                   | Al                                       | Cu    | Steel | Stain-<br>less<br>steel | Ti    |       |
| 1,1'-binaphthyl (A) <sup>3</sup>                     | 0.20                                 | 3733-45               | -2.6                           | -----                  | -----                                       | -----             | -----                                       | -----                    | Dark brown<br>gel.                | -----                                    | ----- | ----- | -----                   | ----- | ----- |
| 1,2-benzanthracene<br>(A).                           | 0.20                                 | 3733-43               | -0.5                           | 137                    | 118                                         | 44                | 120                                         | 2.6                      | Dark brown                        | -----                                    | ----- | ----- | -----                   | ----- | ----- |
| Benzo(a)pyrene<br>(EK).                              | 0.20                                 | 3751-9                | -0.7                           | 133                    | 111                                         | 42                | 110                                         | 4.2                      | do                                | +0.10                                    | -0.04 | +0.10 | +0.02                   | +0.02 | ----- |
|                                                      | 0.20                                 | 3751-2                | -0.5                           | 89                     | 41                                          | 29                | 45                                          | 4.4                      | do                                | +0.30                                    | -0.30 | +0.08 | +0.06                   | +0.04 | ----- |
|                                                      | 0.20                                 | 3751-14               | 0.0                            | 86                     | 36                                          | 28                | 40                                          | 4.7                      | do                                | -----                                    | ----- | ----- | -----                   | ----- | ----- |
| 4,4'-bis(dimethyl-<br>amino) benzopheno-<br>ne (EK). | 0.05                                 | 3893-21               | -1.1                           | -----                  | -----                                       | -----             | -----                                       | -----                    | Brown gel                         | -----                                    | ----- | ----- | -----                   | ----- | ----- |
|                                                      | 0.05                                 | 3893-29               | -2.0                           | -----                  | -----                                       | -----             | -----                                       | -----                    | Dark brown<br>gel.                | -----                                    | ----- | ----- | -----                   | ----- | ----- |
| Chrysene (EK)                                        | 0.03                                 | 3893-21               | -1.9                           | -----                  | -----                                       | -----             | -----                                       | -----                    | do                                | -----                                    | ----- | ----- | -----                   | ----- | ----- |
|                                                      | 0.03                                 | 3893-28               | -4.6                           | -----                  | -----                                       | -----             | -----                                       | -----                    | do                                | -----                                    | ----- | ----- | -----                   | ----- | ----- |
| 2,5-diphenyloxazole<br>(EK).                         | 0.50                                 | 3892-22               | -0.8                           | -----                  | -----                                       | -----             | -----                                       | -----                    | do                                | -----                                    | ----- | ----- | -----                   | ----- | ----- |
|                                                      | 0.50                                 | 3893-29               | -0.6                           | -----                  | -----                                       | -----             | -----                                       | -----                    | do                                | -----                                    | ----- | ----- | -----                   | ----- | ----- |
| Fluoranthene<br>(RTCC).                              | 0.50                                 | 3893-23               | -1.1                           | -----                  | -----                                       | -----             | -----                                       | -----                    | Viscous brown                     | -----                                    | ----- | ----- | -----                   | ----- | ----- |
|                                                      | 0.50                                 | 3893-29               | -0.9                           | >500                   | >733                                        | (6)               | (6)                                         | 1.6                      | Clear, dark<br>brown.             | +0.6                                     | -0.52 | +0.02 | 0.00                    | +0.02 | ----- |
| Pyrene (CCC)                                         | 0.10                                 | 3893-24               | -1.0                           | 201                    | 235                                         | 33                | 65                                          | 2.0                      | Clear, brown                      | -----                                    | ----- | ----- | -----                   | ----- | ----- |
|                                                      | 0.10                                 | 3893-30               | -0.9                           | 431                    | 618                                         | 249               | 1,145                                       | 1.7                      | Clear, dark<br>brown.             | -----                                    | ----- | ----- | -----                   | ----- | ----- |
| Phenanthrene<br>(CCC).                               | 1.00                                 | 3893-25               | -1.6                           | -----                  | -----                                       | -----             | -----                                       | -----                    | Viscous, brown                    | -----                                    | ----- | ----- | -----                   | ----- | ----- |
|                                                      | 1.00                                 | 3893-30               | -1.4                           | -----                  | -----                                       | -----             | -----                                       | -----                    | do                                | -----                                    | ----- | ----- | -----                   | ----- | ----- |
| Acenaphthene<br>(EK) <sup>4</sup>                    | 1.00                                 | 3893-26               | -0.7                           | 124                    | 106                                         | 43                | 115                                         | 2.6                      | Brown gel                         | +0.10                                    | -0.90 | +0.10 | +0.08                   | +0.04 | ----- |
|                                                      | 1.00                                 | 3893-30               | -0.6                           | 114                    | 90                                          | 39                | 95                                          | 2.5                      | Opaque, brown.                    | -----                                    | ----- | ----- | -----                   | ----- | ----- |

<sup>1</sup> Viscosity of the F-50 silicone fluid before test was 60 cs. at 100° F. and 20 cs. at 210° F.

<sup>2</sup> Acid number was determined by the procedure given in Scott, Standard Methods of Chemical Analysis, vol. II, page 1844, 5th Ed., 1939, Van Nostrand Co., Inc., N.Y.

<sup>3</sup> A=Aldrich Chemical Co.; EK=Eastman Kodak; RTCC=Reilly Tar and Chemical Co.; CCC=Carbide and Carbon Chemicals Co.

<sup>4</sup> 1.3 mg. petroleum ether insolubles recovered 3893-26.

<sup>5</sup> Insufficient sample.

Table VI

THE MOST EFFECTIVE ADDITIVES IN F-50 SILICONE FLUID AT 518° F., 1 LITER DRY AIR/HOUR FOR 48 HOURS

| Additive 0.2% concentration                        | Note-book page                                                              | Solubility <sup>1</sup> in fluid                                                                               | Fluid wt. change (g.)                                | Viscosity <sup>2</sup>                    |                                         | Acid <sup>3</sup> No.                         | Appearance of fluid after test                                                                        | Change in metals (mg./cm. <sup>2</sup> )                    |                                                             |                                                             |                                                             |                                            |
|----------------------------------------------------|-----------------------------------------------------------------------------|----------------------------------------------------------------------------------------------------------------|------------------------------------------------------|-------------------------------------------|-----------------------------------------|-----------------------------------------------|-------------------------------------------------------------------------------------------------------|-------------------------------------------------------------|-------------------------------------------------------------|-------------------------------------------------------------|-------------------------------------------------------------|--------------------------------------------|
|                                                    |                                                                             |                                                                                                                |                                                      | cs. at 100° F.                            | Percent Visc. change at 100° F.         |                                               |                                                                                                       | Al                                                          | Cu                                                          | Steel                                                       | Ag                                                          | Ti                                         |
| 1,1'-binaphthyl (A) <sup>4</sup>                   | (3321-4)<br>(3363-43)                                                       | Soluble.....<br>Almost completely soluble.....                                                                 | +0.1<br>-1.0                                         | 130<br>84                                 | 107<br>33                               | 1.7<br>1.5                                    | Clear, yellow.....<br>Clear, dark yellow.....                                                         | 0.00<br>+0.04                                               | -0.78<br>-0.48                                              | +0.16<br>0.00                                               | +0.28<br>+0.32                                              | -0.06                                      |
| Decacyclene (A) <sup>5</sup>                       | 3438-44<br>(3321-20)<br>3368-44<br>3438-45<br>3438-49<br>3321-23<br>3363-45 | do.....<br>Partially soluble.....<br>do.....<br>Insoluble.....<br>do.....<br>Partially soluble.....<br>do..... | -1.1<br>-0.6<br>-0.5<br>-0.7<br>-0.3<br>-0.4<br>+0.1 | 137<br>94<br>120<br>101<br>88<br>73<br>64 | 118<br>49<br>91<br>60<br>40<br>35<br>27 | 1.8<br>1.1<br>2.7<br>2.0<br>1.7<br>1.9<br>1.8 | do.....<br>Brown.....<br>Opaque, brown.....<br>do.....<br>do.....<br>Yellow.....<br>Clear, brown..... | +3.08<br>+0.48<br>-0.06<br>-2.82<br>+0.14<br>+0.70<br>+0.08 | -1.36<br>+0.16<br>-0.20<br>-0.20<br>-0.26<br>-1.12<br>-2.10 | +0.86<br>+0.30<br>-0.10<br>-0.64<br>+0.06<br>+0.24<br>-0.04 | -4.78<br>+0.38<br>+0.02<br>-5.42<br>+0.24<br>+0.40<br>+0.18 | +10.0<br>+10.06<br>-0.20<br>-9.88<br>+0.08 |
| 1,2-benzanthracene (A)                             | 3438-6                                                                      | Almost completely soluble.....                                                                                 | -0.4                                                 | 64                                        | 2.7                                     | 1.8                                           | Clear, dark yellow.....                                                                               | +0.28                                                       | -0.76                                                       | +0.04                                                       | +0.20                                                       | +0.60                                      |
| Dinaphthylene-thiophene (A) <sup>5</sup>           | 3321-25<br>3368-46<br>3438-43<br>3438-49<br>3490-1                          | Partially soluble.....<br>do.....<br>do.....<br>do.....<br>do.....                                             | -0.4<br>+0.8<br>-0.4<br>-0.2<br>-0.2                 | 83<br>73<br>70<br>59<br>56                | 33<br>16<br>11<br>6                     | 1.2<br>2.2<br>1.4<br>1.9<br>1.1               | Brown.....<br>Opaque, brown.....<br>Opaque, brown.....<br>Clear, brown.....<br>Clear, yellow.....     | +0.20<br>+0.02<br>+0.12<br>+0.12<br>+0.08                   | +0.14<br>-0.52<br>-0.12<br>-0.06<br>-0.26                   | +0.22<br>+0.08<br>+0.10<br>+0.04<br>+0.12                   | +0.30<br>+0.02<br>+0.10<br>+0.08<br>+0.06                   | -                                          |
| 4,4'-bis(dimethylamino)-benzophenone (EK)          | 3368-47<br>3438-5<br>3438-42<br>3438-50<br>3321-44                          | Insoluble.....<br>do.....<br>do.....<br>do.....<br>do.....                                                     | -0.9<br>-0.06<br>-1.1<br>-0.7<br>-1.1                | 117<br>193<br>91<br>155<br>104            | 86<br>207<br>44<br>146<br>65            | 0.8<br>0.8                                    | do.....<br>do.....<br>Opaque, yellow.....<br>Clouded, yellow.....<br>Yellow.....                      | +0.08<br>+0.06<br>+0.18<br>+0.24<br>+0.02                   | -0.26<br>-0.28<br>-0.02<br>-0.14<br>-0.12                   | +0.12<br>+0.12<br>+0.16<br>+0.38<br>+0.08                   | +0.20<br>+0.24<br>+0.14<br>+0.28<br>+0.26                   | +0.02<br>-0.02<br>+0.10<br>+0.10<br>-      |
| Chrysene (EK)                                      | 3438-4                                                                      | do.....                                                                                                        | -0.5                                                 | 108                                       | 71                                      | 1.4                                           | Clear, yellow.....                                                                                    | +0.16                                                       | -0.16                                                       | -0.02                                                       | +0.22                                                       | -0.02                                      |
| N,N'-di-2-naphthyl-p-phenylenediamine (EK)         | 3368-24<br>3438-46                                                          | do.....<br>do.....                                                                                             | -0.4<br>-0.2                                         | 71<br>70                                  | 13<br>11                                | 0.8<br>0.6                                    | Opaque, brown.....<br>do.....                                                                         | +2.66<br>+0.04                                              | -0.92<br>-0.54                                              | +0.74<br>+0.10                                              | -3.14<br>+0.10                                              | -                                          |
| Indanthrene Navy Blue BRA powder (GD) <sup>5</sup> | 3368-33<br>3438-48<br>3368-39                                               | Partially soluble.....<br>Insoluble.....<br>Almost completely soluble.....                                     | -1.2<br>-0.6<br>-1.1                                 | 90<br>136<br>162                          | 44<br>116<br>157                        | 2.5<br>1.8<br>1.5                             | Violet.....<br>Clear, violet.....<br>Yellow.....                                                      | +0.02<br>+0.28<br>+0.02                                     | -1.98<br>-0.08<br>-0.64                                     | -0.02<br>+0.06<br>-0.04                                     | +0.40<br>+0.30<br>+0.26                                     | 0.00                                       |
| 2,5-diphenyloxazole (EK)                           | 3438-40<br>3490-26<br>3490-27<br>3893-11<br>3893-11<br>3438-16              | do.....<br>do.....<br>do.....<br>do.....<br>do.....<br>do.....                                                 | -0.5<br>-0.4<br>-0.5<br>-0.1<br>-0.3<br>-0.7         | 66<br>84<br>69<br>97<br>119<br>88         | 5<br>33<br>9.8<br>61<br>98<br>40        | 1.5<br>1.7<br>1.7<br>1.4<br>1.2<br>1.8        | Clear, yellow.....<br>do.....<br>do.....<br>do.....<br>do.....<br>do.....                             | +0.06<br>+0.06<br>+0.02<br>+0.02                            | -0.46<br>-0.28<br>-0.42<br>-0.42                            | +0.04<br>+0.06<br>+0.02<br>+0.02                            | +0.22<br>+0.24<br>+0.20<br>+0.00                            | +0.06                                      |
| Fluoranthene (RTCC)                                | 3438-16<br>3490-25<br>3490-42<br>3608-42<br>3608-10<br>3557-44              | do.....<br>do.....<br>do.....<br>do.....<br>do.....<br>do.....                                                 | -0.4<br>-0.4<br>-0.7<br>-0.8<br>-0.5<br>-0.3         | 187<br>117<br>108<br>82<br>79<br>73       | 197<br>85<br>73<br>30<br>25<br>27       | 1.5<br>1.2<br>2.7<br>2.4<br>2.1<br>do.....    | do.....<br>do.....<br>do.....<br>do.....<br>Clear, red.....<br>do.....                                | +0.08<br>+0.06<br>+0.06<br>+0.04<br>+0.08<br>+0.06          | -0.12<br>-0.22<br>-0.24<br>-0.02<br>-0.06<br>-0.24          | +0.08<br>+0.22<br>+0.00<br>+0.02<br>+0.10<br>0.00           | +0.42<br>+0.38<br>+0.22<br>+0.26<br>+0.02<br>+0.02          | +0.02                                      |
| Fluoranthene (CCC)                                 | 3557-42<br>3608-30<br>3608-50<br>3557-45<br>3608-31                         | Partially soluble.....<br>Partially soluble.....<br>do.....<br>do.....<br>Insoluble.....                       | -0.5<br>-0.2<br>-0.3<br>-0.4<br>-0.4                 | 82<br>73<br>73<br>76<br>72                | 30<br>16<br>15<br>20<br>14              | 2.4<br>3.1<br>2.8<br>2.1<br>3.0               | do.....<br>Clear, brown.....<br>do.....<br>Clear, red.....<br>Clear, brown.....                       | +0.04<br>+0.02<br>+0.08<br>+0.04<br>+0.06                   | -0.02<br>+0.20<br>+0.40<br>+0.34<br>-0.32                   | +0.08<br>+0.10<br>+0.00<br>+0.08<br>+0.10                   | +0.26<br>+0.10<br>+0.14<br>+0.16<br>+0.02                   | +0.02                                      |
| Perylene (A)                                       | 3608-49<br>3627-1<br>3557-46<br>3608-32                                     | do.....<br>Partially soluble.....<br>do.....<br>do.....                                                        | -0.3<br>-0.3<br>+0.6<br>-0.3                         | 73<br>73<br>71<br>58                      | 16<br>13<br>13<br>-7.6                  | 2.8<br>2.3<br>3.2                             | do.....<br>do.....<br>Clear, yellow.....<br>Clear, light brown.....                                   | +0.04<br>+0.12<br>+0.12<br>+0.06                            | +0.22<br>+0.28<br>+0.28<br>-0.18                            | +0.04<br>+0.06<br>+0.06<br>+0.08                            | +0.12<br>+0.18<br>+0.18<br>+0.10                            | 0.00                                       |
| Benzo(a)pyrene (EK)                                | 3608-49<br>3627-1<br>3557-46<br>3608-31                                     | do.....<br>Partially soluble.....<br>do.....<br>Insoluble.....                                                 | -0.3<br>-0.3<br>+0.6<br>-0.4                         | 73<br>73<br>71<br>72                      | 16<br>13<br>13<br>14                    | 2.8<br>2.3<br>3.0                             | do.....<br>do.....<br>do.....<br>Clear, brown.....                                                    | +0.04<br>+0.04<br>+0.04<br>+0.06                            | +0.22<br>+0.28<br>+0.34<br>-0.32                            | +0.04<br>+0.06<br>+0.08<br>+0.10                            | +0.02<br>+0.02<br>+0.02<br>+0.02                            | 0.00                                       |
| Dibenz(a, h)anthracene (EK)                        | 3608-49<br>3608-8<br>3608-9                                                 | do.....<br>Partially soluble.....<br>Almost completely soluble.....                                            | 0.0<br>-0.1<br>-1.8                                  | 76<br>89<br>91                            | 21<br>41<br>43                          | 2.9<br>2.5<br>2.5                             | do.....<br>Clear, brown.....<br>do.....                                                               | +0.06<br>+0.06<br>+0.04                                     | +0.20<br>-0.42<br>-0.06                                     | +0.02<br>+0.04<br>+0.08                                     | +0.12<br>+0.22<br>+0.26                                     | 0.00                                       |
| Pyrene (EK)                                        | 3608-11<br>3608-33<br>3627-2<br>3608-43                                     | Soluble.....<br>do.....<br>do.....<br>Almost completely soluble.....                                           | -1.1<br>-0.7<br>-1.1<br>-0.5                         | 108<br>81<br>137<br>113                   | 60<br>28<br>118<br>79                   | 2.0<br>2.7<br>2.1<br>2.8                      | Clear, yellow.....<br>do.....<br>do.....<br>Clear, light brown.....                                   | +0.26<br>+0.08<br>+0.12<br>+0.10                            | -0.36<br>-0.84<br>-0.10<br>+0.36                            | +0.08<br>+0.06<br>+0.04<br>+0.08                            | +0.32<br>+0.24<br>+0.06<br>+0.32                            | 0.00                                       |
| Phenanthrene (CCC)                                 | 3608-11<br>3608-33<br>3627-2<br>3608-43                                     | do.....<br>do.....<br>do.....<br>do.....                                                                       | -1.1<br>-0.7<br>-1.1<br>-0.5                         | 108<br>81<br>137<br>113                   | 60<br>28<br>118<br>79                   | 2.0<br>2.7<br>2.1<br>2.8                      | do.....<br>do.....<br>do.....<br>Clear, light brown.....                                              | +0.26<br>+0.08<br>+0.12<br>+0.10                            | -0.36<br>-0.84<br>-0.10<br>+0.36                            | +0.08<br>+0.06<br>+0.04<br>+0.08                            | +0.32<br>+0.24<br>+0.06<br>+0.32                            | 0.00                                       |
| Acenaphthene (EK)                                  | 3608-48<br>3490-13<br>3490-22<br>3557-43                                    | Partially soluble.....<br>Insoluble.....<br>do.....<br>do.....                                                 | -0.9<br>-0.9<br>-0.3<br>-0.7                         | 146<br>70<br>69<br>139                    | 132<br>11<br>9.8<br>121                 | 2.5<br>0.3<br>0.3<br>1.0                      | do.....<br>Opaque, brown.....<br>Clear, brown.....<br>Opaque, brown.....                              | +0.02<br>+0.02<br>+0.08<br>+0.12                            | +1.24<br>-0.52<br>-2.42<br>-0.12                            | +0.06<br>+0.06<br>+0.08<br>+0.12                            | +0.40<br>+0.02<br>+0.10<br>+0.20                            | 0.00<br>0.00<br>+0.04<br>0.02              |

<sup>1</sup> The additive (0.040 g.) was placed in the test tube and 20 ml. of the test fluid was added. The inlet tube (on which the washers were spaced) was inserted, and the test tube was heated on a steam bath for 5 minutes while nitrogen was bubbled through the inlet tube to provide agitation. Solubility was estimated after standing at room temperature for about an hour. Metal washers were handled in accordance with Appendix I of WADC Technical Report 55-449, Part 3, dated May 1956.

<sup>2</sup> Viscosity of F-50 silicone fluid before test was 62.8 cs. at 100° F.

<sup>3</sup> Acid number was determined by the procedure given in Scott, Standard Methods of Chemical Analysis, vol. II, page 1844, 5th ed., 1939, D. Van Nostrand Co., Inc., N.Y.

<sup>4</sup> A=Aldrich Chemical Co.; EK=Eastman Kodak; GD=General Dyestuff Co.; RTCC=Reilly Tar and Chemical Corp.; CCC=Carbide and Carbon Chemicals Co.; WADC=Wright Air Development Center.

<sup>5</sup> Small amount of petroleum ether insoluble residue after test.

| Decacyclene:                                | (3438-45) | (3438-49) | (3438-49) | (3438-49) | (3438-49) | (3438-49) | (3438-49) | (3438-49) | (3438-49) | (3438-49) | (3438-49) | (3438-49) |
|---------------------------------------------|-----------|-----------|-----------|-----------|-----------|-----------|-----------|-----------|-----------|-----------|-----------|-----------|
|                                             | (3438-45) |           |           |           |           |           |           |           |           |           |           |           |
|                                             | (3438-49) |           |           |           |           |           |           |           |           |           |           |           |
|                                             |           |           |           |           |           |           |           |           |           |           |           |           |
| Dinaphthylene-thiophene:                    |           |           |           |           |           |           |           |           |           |           |           |           |
|                                             | (3438-43) |           |           |           |           |           |           |           |           |           |           |           |
|                                             | (3438-49) |           |           |           |           |           |           |           |           |           |           |           |
|                                             |           |           |           |           |           |           |           |           |           |           |           |           |
| Indanthrene Navy Blue BRA powder: (3438-48) |           |           |           |           |           |           |           |           |           |           |           |           |
|                                             |           |           |           |           |           |           |           |           |           |           |           |           |
| N-phenylferrocene-carboxamide:              |           |           |           |           |           |           |           |           |           |           |           |           |
|                                             | (3490-22) |           |           |           |           |           |           |           |           |           |           |           |
|                                             | (3490-13) |           |           |           |           |           |           |           |           |           |           |           |
|                                             |           |           |           |           |           |           |           |           |           |           |           |           |
| (3557-43)                                   |           |           |           |           |           |           |           |           |           |           |           |           |

On the basis of effectiveness and solubility alone, the best additive is: benzo(a)pyrene. Unfortunately, it is a powerful carcinogenic agent. Dibenz(a,h)anthracene is also very effective, though quite insoluble at low temperatures.

In an attempt to determine the phenomena involved in the gelation of silicone fluids and inhibition of the same

70 in the presence of the antioxidant materials of this invention, further experiments were conducted on the F-50 silicone oil. Fluoranthene was chosen as the antioxidant for study because of its efficacy, solubility, non-carcinogenic character and easy detection in the ultraviolet.

The silicone fluid to be tested was brought to gelation by bubbling a stream of air through 20 gram samples of

the fluid heated in tubes at 518° F. The time required for gelation of the oil under the various conditions tested served as the most apparent indication of the rate and extent of oxidative degradation. The degree of chemical change in the fluid itself, up to the point of gelation, was not large enough to be detected by comparison of infrared spectra and, for this reason, the data most pertinent to the oxidation process involved a determination of the by-products formed from the reaction.

During the reaction leading to gelation, oxygen was consumed and a number of volatile products were evolved and carried out of the sample tubes in the air stream. The volatile products identified and determined quantitatively included formaldehyde, formic acid, carbon dioxide, carbon monoxide, water, cyclic siloxanes and tetrachlorobenzene. In order to collect the condensable volatile products, the exit gases from 6 samples of fluid (20 grams each) were lead through a manifold into a trap immersed in a Dry-Ice acetone bath and the resultant products were analyzed quantitatively.

In experiments in which the silicone fluid contained fluoranthene, 9-fluorenone-1-carboxylic acid and recovered fluoranthene were obtained. The oxygen consumption was calculated from the overall weight increase and this was compared with the amount of oxygen removed from the air stream. The rate of oxygen taken up and of carbon monoxide and carbon dioxide evolved were also determined for the entire reaction period. The comparison of all these factors were made for unprotected fluid and fluid containing 0.2 percent fluoranthene. The test results obtained on gelation inhibition are set forth in Table VII.

10

assumption that all the products of methyl cleavage were volatilized and determined. It is seen that the number of methyls removed is only slightly larger (2.83) in the presence of the additive than for unprotected fluid (2.60), although the time was increased sevenfold. Since each molecule contains an average of 82 methyl groups, about  $\frac{1}{30}$  of the methyl groups was lost:

|                          | Unprotected fluid     | Protected fluid       |
|--------------------------|-----------------------|-----------------------|
| Methyls cleaved/molecule | $2.60 = \frac{1}{30}$ | $2.83 = \frac{1}{30}$ |
| Total methyls/molecule   | 82 = 32               | 82 = 29               |

15

The presence of 0.2 percent fluoranthene in protected fluid amounted to 1 molecule per 33 molecules of silicone polymer, or 1 fluoranthene molecule per 2700 methyls. Of these 2700 methyls about 93 were lost during oxidative gelation. Tetrachlorophenyl cleavage was relatively unimportant, about 1 group from 100 silicone molecules. Each silicone molecule contained an average of 1.5 tetrachlorophenyl groups.

20

The number of moles of oxygen consumed per mole of fluid up to gel point, as determined by metering the oxygen content of the exit gases, can be checked in two ways. Although the fluid itself undergoes a weight loss during the oxidation due to loss of volatile products, there is an overall weight increase when all the products are determined. This increase must be due only to the oxygen taken up by the fluid, and its magnitude must be equivalent to the amount of oxygen. Another check can

Table VII  
OXIDATION OF F-50 SILICONE FLUID AT 518° F. TO GEL POINT

| Experiment                      | Without additive |       |       |       |                 | Containing 0.2% additive |       |       |       |                 |
|---------------------------------|------------------|-------|-------|-------|-----------------|--------------------------|-------|-------|-------|-----------------|
|                                 | A                | B     | C     | D     | Average         | E                        | F     | G     | H     | Average         |
| Wt. fluid (g.)                  | 120.6            | 120.6 | 120.4 | 120.5 | $120.5 \pm 0.1$ | 120.9                    | 122.0 | 120.4 | 121.2 | $121.1 \pm 0.5$ |
| Fluoranthene added (g.)         | None             | None  | None  | None  | None            | 0.240                    | 0.240 | 0.240 | 0.240 | 0.240           |
| Gel time (hrs.)                 | 10.2             | 10.9  | 10.2  | 10.2  | $10.4 \pm 0.3$  | 72                       | 73    | 70    | 70    | $71 \pm 1$      |
| HCHO (g.)                       | 1.90             | 1.94  | 1.96  | 1.90  | $1.93 \pm 0.02$ | 2.23                     | 2.31  | 2.23  | 2.23  | $2.26 \pm 0.04$ |
| HCOOH (g.)                      | 0.722            | 0.588 | 0.637 | 0.637 | $0.63 \pm 0.09$ | 0.422                    | 0.376 | 0.65  | 0.65  | $0.48 \pm 0.10$ |
| H <sub>2</sub> O (g.)           | 0.98             | 0.91  | 0.98  | 0.98  | $0.94 \pm 0.04$ | 1.97                     | 2.21  | 2.21  | 2.21  | $2.09 \pm 0.12$ |
| CO (g.)                         |                  |       |       |       | 0.60            | 0.60                     | 0.60  | 0.60  | 0.60  | 0.60            |
| CO <sub>2</sub> (g.)            | 0.233            | 0.249 | 0.233 | 0.233 | 0.233           | 0.241 $\pm 0.008$        | 0.044 | 0.100 | 0.097 | 0.097           |
| Tetrachlorobenzene (g.)         | 0.080            | 0.105 | 0.080 | 0.080 | 0.080           | 0.092 $\pm 0.012$        | 0.098 | 0.088 | 0.088 | 0.088           |
| Siloxanes (g.)                  | 1.59             | 1.88  | 1.59  | 1.59  | 1.79 $\pm 0.15$ | 2.94                     | 3.67  | 3.15  | 3.15  | 3.25 $\pm 0.40$ |
| Fluoranthene recovered:         |                  |       |       |       |                 |                          |       |       |       |                 |
| In condensate (g.)              |                  |       |       |       |                 |                          |       |       |       |                 |
| In gel (g.)                     |                  |       |       |       |                 |                          |       |       |       |                 |
| Total condensable products (g.) | 6.63             | 6.27  | 6.50  | 6.50  | 6.47 $\pm 0.13$ | 8.03                     | 8.93  | 9.81  | 9.81  | 9.92 $\pm 0.60$ |
| Total volatile products (g.)    |                  |       |       |       |                 |                          |       |       |       |                 |
| Wt. loss of fluid (g.)          | 3.7              | 3.1   | 3.7   | 3.7   | 3.5 $\pm 0.3$   | 3.85                     | 5.28  | 6.12  | 6.12  | 9.75 $\pm 0.6$  |
| Over-all wt. increase (g.)      |                  |       |       |       |                 |                          |       |       |       |                 |
| Metered O <sub>2</sub> uptake:  |                  |       |       |       |                 |                          |       |       |       |                 |
| (G.)                            | 3.10             | 3.26  | 2.85  | 2.85  | 3.07 $\pm 0.15$ | 4.80                     | 4.80  | 4.64  | 4.64  | 4.72 $\pm 0.08$ |
| Percent of total available.     | 18.7             | 18.5  | 17.5  | 17.5  | 18.2 $\pm 0.5$  | 4.1                      | 4.1   | 4.1   | 4.1   | 4.1             |

The test results on gelation inhibition, as set forth in Table VII, give gram quantities of the various products formed and the amounts of oxygen consumed up to the gel point. The molar ratios of these products to one mole of silicone fluid were calculated from the averages and are compiled as follows:

| Volatile products     | Molar ratios without additive | Molar ratios with 0.2% additive |
|-----------------------|-------------------------------|---------------------------------|
| HCHO                  | 1.60                          | 1.86                            |
| HCOOH                 | .34                           | .26                             |
| H <sub>2</sub> O      | 1.29                          | 2.88                            |
| CO                    | .52                           | .67                             |
| CO <sub>2</sub>       | .14                           | .045                            |
| Tetrachlorobenzene    | .0106                         | .0105                           |
| Methyl groups cleaved | 2.60                          | 2.83                            |

The number of methyl groups cleaved per molecule of silicone fluid was calculated by adding up the molar ratios of the carbon-containing products from the oxidation of methyl groups. This calculation involves the reasonable

be obtained by adding up the number of oxygen atoms which appear in the products of the reaction from 1 mole of silicone fluid. This amounts to all the oxygens in the volatile products plus  $\frac{1}{2}$  an oxygen atom for each methyl group cleaved, on the assumption that each methyl group removed from a silicone atom is replaced by a siloxane link. The total number of oxygen atoms is then equal to twice the moles of oxygen consumed. The molar ratios of oxygen consumed by 1 mole of silicone fluid determined by these three methods are compared as follows:

| Oxygen consumed                 | Unprotected fluid | Protected fluid |
|---------------------------------|-------------------|-----------------|
| Metered O <sub>2</sub> uptake   | 2.39              | 3.63            |
| Calcd. from weight increase     | 2.96              | 3.61            |
| Calcd. from O atoms in products | 2.83              | 3.72            |
| Averages                        | 2.73 $\pm$ .22    | 3.65 $\pm$ .04  |

75

Averages of the three methods are seen to be  $2.73 \pm 0.22$  moles of oxygen per mole of unprotected fluid and  $3.65 \pm 0.04$  moles of oxygen per mole of fluid containing fluoranthene.

It appears that gelation of a silicone fluid depends on cleavage of methyl groups from the fluid and this apparently leads to crosslinking of silicone molecules. Tetrachlorobenzene is a very minor product of the oxidation process and the loss of tetrachlorophenyl groups (one from 100 silicone molecules) can in no way account for the gelation of the fluid. The action of the additives seems to be only to delay oxygen pickup, methyl cleavage and crosslinking rather than to change the nature of the chemical reactions involved. This delaying action must occur before cleavage of the Si-C bond since oxygen consumption and methyl cleavage are affected. It is reasonable to assume that the crosslinks formed are merely additional siloxane bonds (Si—O—Si) between the linear silicone molecules, since no new type of bonds were detected by infrared comparison of unoxidized and gelled fluid.

From an examination of the foregoing, it will be seen that the instant invention provides silicone lubricants which are especially amenable for use in present day high speed propulsion devices. The flat viscosity temperature curves exhibited by these lubricants as well as their oxidation stability at elevated temperatures makes them highly advantageous for use in devices which encounter wide ranges of temperatures during their operation.

The term percent as used in the instant specification and appended claim refers to percent by weight unless otherwise indicated. It is to be further understood that although the compositions described herein illustrate a preferred form of the invention, modifications and alterations can be made by those skilled in the art without departing from the spirit and scope thereof, and that all such modifications as fall within the scope of the appended claim are intended to be included herein.

What is claimed is:

A lubricating fluid composition comprising a silicone oil and, as a gelation inhibitor, from about 0.2 percent to about 2.0 percent by weight of 2,5-diphenyloxazole.

References Cited in the file of this patent

UNITED STATES PATENTS

|           |                |       |                |
|-----------|----------------|-------|----------------|
| 1,761,810 | Bjerregaard    | ----- | June 3, 1930   |
| 1,904,433 | Fischer et al. | ----- | Apr. 18, 1933  |
| 1,918,593 | Dow            | ----- | July 18, 1933  |
| 2,191,089 | Barth          | ----- | Feb. 20, 1940  |
| 2,208,105 | Rathbun        | ----- | July 16, 1940  |
| 2,221,953 | Read           | ----- | Nov. 19, 1940  |
| 2,427,766 | Diamond        | ----- | Sept. 23, 1947 |
| 2,491,120 | Loane et al.   | ----- | Dec. 13, 1949  |
| 2,561,178 | Burkhard       | ----- | July 17, 1951  |
| 2,689,859 | Burkhard       | ----- | Sept. 21, 1954 |
| 3,026,263 | Arimoto        | ----- | Mar. 20, 1962  |
| 3,047,501 | Brook et al.   | ----- | July 31, 1962  |

FOREIGN PATENTS

|         |               |       |               |
|---------|---------------|-------|---------------|
| 809,360 | Great Britain | ----- | Feb. 25, 1959 |
|---------|---------------|-------|---------------|